

## UNITED STATES PATENT OFFICE

2,546,167

ACID-FADING INHIBITION USING DIBEN-  
ZYLETHYLENEDIAMINEVictor S. Salvin, Irvington, and John R. Adams,  
Jr., Summit, N. J., assignors to Celanese Cor-  
poration of America, a corporation of DelawareNo Drawing. Application July 3, 1948,  
Serial No. 37,093

13 Claims. (Cl. 8—61)

1

This invention relates to the treatment of dyed organic derivative of cellulose textile materials, and relates more particularly to the treatment of organic derivative of cellulose textile materials dyed with dyestuffs having a tendency to fade when exposed to an acid atmosphere, whereby said fading is inhibited.

An object of this invention is to provide an improved process for the treatment of colored cellulose acetate or other organic derivative of cellulose textile materials which have been dyed with colors which are not ordinarily fast to acid fumes whereby the resistance of said dyed textile materials to acid fading is substantially improved.

Another object of this invention is the provision of dyed cellulose acetate or other organic derivative of cellulose textile materials which are highly resistant to acid fading.

A further object of this invention is the production of dyed cellulose acetate or other organic derivative of cellulose textile materials having acid fading inhibitors incorporated therein which have a substantive affinity for said cellulose acetate or other organic derivative of cellulose textile materials and which do not dissolve when said treated materials are exposed to light and to acid fumes.

Other objects of this invention will appear from the following detailed description.

In the coloration of textile materials it is very desirable that the colors produced on the materials be as fast as possible to light, washing, and to other agencies such as acid fumes. Many dyestuffs yield on organic derivative of cellulose materials desirable colors which are fast to washing but these colors often suffer from a lack of fastness to acid fumes. When fabrics to which these dyestuffs have been applied are exposed to acid fumes, such as, for example, the products of combustion of coal, gas, etc., the color undergoes a change in shade. This change is usually referred to as acid fading. The change which occurs may be a dulling of the brightness of the shade in some instances, and in others there may be a definite change in color. This undesirable effect is frequently observed in the case of many anthraquinone dyestuffs which yield valuable blue colors on organic derivative of cellulose materials. When fabrics dyed with these colors are exposed to acid fumes the colors change from a pure blue shade to one having a reddish cast. On continued exposure to the acid fumes the blue color may even change to a pink color. Such changes naturally restrict the range of usefulness of these dyestuffs. Accordingly, methods of increasing the resistance of these dyes to acid fading are of great commercial importance.

We have now found that the acid fading characteristics of dyed cellulose acetate or other organic derivative of cellulose textile materials

which have been dyed with dyestuffs which are not fast to the action of acid fumes may be substantially improved if there is applied to said dyed cellulose acetate or other organic derivative of cellulose textile material an amine selected from the group consisting of diphenylbenzamidine and dibenzylethylenediamine. Each of said amines have a substantive affinity for cellulose acetate or other organic derivative of cellulose and are water insoluble so that they are unaffected by washing. Furthermore, they are strongly resistant to any changes under the action of acid fumes and, accordingly, do not discolor. While said amine acid fading inhibiting agents may be applied to the dyed cellulose acetate or other organic derivative of cellulose textile material in the form of a solution in a solvent such as aqueous alcohol, diacetone alcohol, or other solvent which does not have an undesirable solvent action on the organic derivative of cellulose material, the most advantageous results are obtained when the amine employed is applied in the form of a stable aqueous emulsion consisting of a solution of said amine in a water-insoluble organic solvent, for example, toluene containing some ethyl alcohol, which is dispersed in water with the aid of suitable dispersing agents to form the desired emulsion, the droplets of the water-insoluble solvent solution of the inhibiting agent comprising the disperse phase and the water the continuous phase of the emulsion.

The emulsion or solution of inhibiting agent is preferably applied to the dyed organic derivative of cellulose textile material by padding operations, the nip of the padding mangle being so adjusted that sufficient liquid is retained on the fabric to deposit in a uniform fashion thereon from 0.3 to 1.0% on the weight of the fabric of the inhibiting agent after the liquid vehicle is removed and the treated fabric is dried. Drying of the padded fabric may be conveniently effected at a temperature of 70 to 150° C., preferably about 85° C., the treated fabric being exposed to said temperature until the liquid present is evaporated, usually in from about 5 to 20 minutes.

When applying diphenylbenzamidine or dibenzylethylenediamine to the dyed textile material in emulsion form, the amine employed is preferably dissolved in a water-insoluble organic liquid solvent therefor containing a plurality of dispersing agents at least one of which is a water-soluble anionic surface active agent and one which is a water-insoluble, but oil-soluble non-ionic surface active agent, and the organic solution obtained then dispersed in water with agitation to form the desired stable aqueous emulsion. The emulsion thus obtained comprises a dispersion of droplets of an organic solution of the inhibitor in water. The water-insoluble but oil-soluble dispersing agent stabilizes the

disperse phase of the emulsion and acts as an auxiliary solvent for the amine inhibitor in the organic solvent while the water-soluble, anionic surface active agent stabilizes the emulsion of the water-insoluble droplets in the aqueous, continuous phase. In treating the textile material, the aqueous emulsion is preferably applied, as stated, by padding operations, although any other convenient method of application may be employed. The method of preparing the 10 novel emulsions is more particularly described in co-pending application S. No. 37,094, filed July 3, 1948.

The application of diphenylbenzamidine or dibenzylethylenediamine as acid fading inhibitors on dyed textile materials and, particularly, in the specific emulsion form in which we preferably apply said inhibitors yields a degree of protection which is quite outstanding. Not only is the degree of protection obtained superior to 20 that obtained when the inhibiting agents are applied, for example, simultaneously with the dyes, but it is also quite superior to the results obtained even when arylamines closely related to said aforementioned amines are employed. We have found that in the case of both diphenylbenzamidine and dibenzylethylenediamine although there are free amino groups present there is a complete absence of the yellowing normally produced when dyed textile materials containing inhibitors having free primary or secondary amino groups are exposed to acid fumes. Consequently, no undesirable modification in shade results on employing either diphenylbenzamidine or dibenzylethylenediamine as an inhibiting 30 agent on the dyed textile materials even after extended exposure of said textile materials to acid fumes. This is quite surprising since many compounds closely related in structure to diphenylbenzamidine and dibenzylethylenediamine discolor appreciably when textile materials having said closely related compounds applied thereto as acid fading inhibitors are exposed to acid fumes. Furthermore, textile materials treated by said emulsion method with dibenzylethylenediamine or diphenylbenzamidine retain their resistance to acid fading even after said materials are washed or subjected to dry cleaning operations.

In order further to illustrate our invention, but without being limited thereto, the following examples are given:

#### Example I

A solution of dispersing agents is formed by dissolving 10 parts by weight of completely sulfonated glyceryl triricinoleate, a water-soluble anionic surface active agent, 10 parts by weight of water miscible, non-ionic monolauryl ether of a polyethylene glycol of the general formula  $\text{HOCH}_2\text{CH}_2-\text{O}(\text{CH}_2\text{CH}_2\text{O})_n-\text{C}_{12}\text{H}_{25}$ , wherein  $n$  is 2 to 10, 10 parts by weight of the dioleate of a polyethylene glycol such as dodecaethyleneglycol which is water-insoluble but oil soluble and non-ionic in character, and 10 parts by weight of dioxan in 60 parts by weight of toluene. 10 parts by weight of dibenzylethylenediamine are dissolved in 30 parts by weight of the above solution by warming the latter to 75 to 80° C. and the resulting solution then poured into 970 parts by weight of water with stirring. An emulsion of organic liquid droplets in water is formed by further stirring at high speed. The average particle size of the amine is thus reduced to about 1 micron or less.

A cellulose acetate fabric dyed in a blue

shade with 1:4-dimethylamino-anthraquinone is padded with the above emulsion, the nip of the padding mangle being so adjusted that the fabric retains an equal weight of liquid. The impregnated fabric is then dried by heating at 80 to 100° C. for about 15 minutes. About 1% on the weight of the dyed fabric of dibenzylethylenediamine is thus incorporated therein. The treated dyed fabric has a resistance to acid fading of 2 units in accordance with the standard A. A. T. C. C. test while untreated dyed fabric has an acid fading resistance of only 0 units. The treated fabric retains its resistance to acid fading even after being washed or dry-cleaned.

#### Example II

An aqueous emulsion containing 1% by weight of diphenylbenzamidine is prepared in the manner described in Example I. When padded onto a cellulose acetate fabric dyed in a blue shade with 1:4-dimethylamino-anthraquinone so as to deposit uniformly thereon 1% by weight of diphenylbenzamidine, the treated dyed fabric obtained exhibits a resistance to acid fading of 25 1.5 units in accordance with the standard A. A. T. C. C. test. As indicated above, untreated dyed fabric has a resistance to acid fading of only 0 units.

#### Example III

To a dyebath comprising an aqueous dispersion containing 0.2% by weight of 1,4-di-methylamino-anthraquinone on the fabric to be dyed is added sufficient diphenylbenzamidine dispersed with the aid of sodium lignosulfonate so that the dyebath contains 1% by weight of the inhibiting agent based on the fabric. The dyebath is raised to a temperature of about 80 to 85° C. and a cellulose acetate fabric is immersed therein for about 1 hour. The fabric is dyed in a blue shade by this treatment and also absorbs about 0.6% by weight based on the fabric of the diphenylbenzamidine. On exposure of the dyed fabric to acid fumes for one unit in accordance with the standard A. A. T. C. C. test, practically no change in shade 30 is observed while after 2 units of exposure the dyed fabric undergoes a slight greying. Cellulose acetate fabric dyed in a similar manner with said dyestuff but without employing diphenylbenzamidine as an acid-fading inhibitor fades to a reddish-purple color after 1 unit of exposure and completely to a pink color after 2 units of exposure. The dyed fabric containing the inhibitor retains its resistance to acid-fading even after washing and dry-cleaning.

#### Example IV

A blue cellulose acetate fabric which has been dyed to a blue shade with 0.3% of 1-amino-4-anilido anthraquinone is padded with a solution 60 of dibenzylethylenediamine in an aqueous alcohol. The composition of the aqueous alcohol is 65% of ethyl alcohol and 35% water by weight. The concentration of the dibenzylethylenediamine in its aqueous alcohol solution is 1% of the weight 65 of the aqueous alcohol solution. The nip of the padding mangle is adjusted so that the fabric contains an equal weight of liquid after it passes through the padding bath at 25° C. The impregnated fabric is then dried to remove the solvent. About 1% of the weight of the dyed fabric of dibenzylethylenediamine is incorporated in this manner within the fabric. Subsequent washing or dry cleaning does not remove the dibenzylethylenediamine and a protective action against

gas fading is not lowered by the washing or dry

cleaning treatments. The treated dyed fabric has a resistance to acid fading of two units in accordance with the standard A. A. T. C. C. test, while untreated dyed fabric has an acid fading resistance of 0 units.

While our invention has been more particularly described in connection with the treatment of textile materials having a basis of cellulose acetate, equally satisfactory results are obtained in the treatment of textile materials having a basis of other organic derivatives of cellulose. Examples of other organic derivatives of cellulose are cellulose esters such as cellulose propionate, cellulose butyrate, cellulose acetate-butyrate and cellulose acetate-propionate and cellulose ethers such as ethyl cellulose and benzyl cellulose.

It is to be understood that the foregoing detailed description is given merely by way of illustration and that many variations may be made therein without departing from the spirit of our invention.

Having described our invention, what we desire to secure by Letters Patent is:

1. Process for improving the fastness of colorations on dyed organic derivative of cellulose textile material to acid fading, which comprises treating said dyed organic derivative of cellulose textile material with dibenzylethylenediamine.

2. Process for improving the fastness of colorations on dyed cellulose acetate textile material to acid fading, which comprises treating said dyed cellulose acetate textile material with dibenzylethylenediamine.

3. Process for improving the fastness of colorations on dyed organic derivative of cellulose textile material to acid fading, which comprises treating said dyed organic derivative of cellulose textile material with a stable emulsion comprising a solution in a water-insoluble organic solvent of dibenzylethylenediamine, which solution is dispersed in water.

4. Process for improving the fastness of colorations on dyed cellulose acetate textile material to acid fading, which comprises treating said dyed cellulose acetate textile material with a stable emulsion comprising a solution in a water-insoluble organic solvent of dibenzylethylenediamine, which solution is dispersed in water.

5. Process for improving the fastness of colorations on dyed organic derivative of cellulose textile materials to acid fading, which comprises treating said dyed organic derivative of cellulose textile materials with a stable emulsion comprising a solution of dibenzylethylenediamine in toluene dispersed in water.

6. Process for improving the fastness of colorations on dyed cellulose acetate textile materials to acid fading, which comprises treating said dyed cellulose acetate textile materials with a stable emulsion comprising a solution of dibenzylethylenediamine in toluene dispersed in water.

7. Process for improving the fastness of colorations on dyed cellulose acetate textile materials to acid fading, which comprises treating said dyed cellulose acetate materials with a stable emulsion comprising a solution of dibenzylethylenediamine in toluene and containing some di-oxan dispersed in water whereby from 0.3 to 1.0% by weight of said amine is applied thereto and then drying the treated material.

8. Process for improving the fastness of colorations on dyed cellulose acetate textile materials to acid fading, which comprises treating said dyed cellulose acetate materials with a stable

emulsion comprising a solution of dibenzylethylenediamine in toluene containing some ethyl alcohol dispersed in water whereby from 0.3 to 1.0% by weight of said amine is applied thereto and then drying the treated textile material.

5. Process for improving the fastness of colorations on dyed cellulose acetate textile material to acid fading, which comprises treating said dyed cellulose acetate textile material with a stable emulsion comprising a solution in a water-insoluble organic solvent of dibenzylethylenediamine dispersed in water, said emulsion being formed by dissolving a plurality of dispersing agents in the organic solvent employed, at least one of which dispersing agents is a water-soluble anionic surface active agent and one a water-insoluble but oil-soluble non-ionic surface active agent, adding the amine thereto, dissolving it therein and dispersing the resulting organic solution in water.

10. Process for improving the fastness of colorations on dyed cellulose acetate textile materials to acid fading, which comprises treating said dyed cellulose acetate textile materials with a stable emulsion comprising a solution of dibenzylethylenediamine in toluene dispersed in water, said emulsion being prepared by dissolving sulfonated glyceryl ricinoleate, a water-insoluble, oil-soluble dioleate of a poly-ethylene glycol

15 and the mono-lauryl ether of a polyethylene glycol in toluene, adding the amine thereto, dissolving it therein, and dispersing the resulting organic solution in water.

11. Dyed organic derivative of cellulose textile material dyed with a dyestuff normally tending to fade on exposure to acid fumes and having incorporated therein dibenzylethylenediamine.

12. Dyed cellulose acetate textile material dyed with a dyestuff normally tending to fade on exposure to acid fumes and having incorporated therein dibenzylethylenediamine.

13. Dyed cellulose acetate textile material dyed with a dyestuff normally tending to fade on exposure to acid fumes and having incorporated therein from 0.3 to 1.0% by weight of dibenzylethylenediamine.

VICTOR S. SALVIN.  
JOHN R. ADAMS, JR.

#### REFERENCES CITED

The following references are of record in the file of this patent:

#### UNITED STATES PATENTS

| Number    | Name    | Date          |
|-----------|---------|---------------|
| 1,690,481 | Ellis   | Nov. 6, 1928  |
| 1,723,271 | Ellis   | Apr. 28, 1931 |
| 1,803,008 | Ellis   | Oct. 18, 1932 |
| 1,883,351 | Dreyfus | Oct. 18, 1932 |
| 2,017,119 | Ellis   | Oct. 15, 1935 |
| 2,083,122 | Olpin   | June 8, 1937  |
| 2,369,122 | Giles   | Feb. 13, 1945 |
| 2,416,380 | Collie  | Feb. 25, 1947 |

#### FOREIGN PATENTS

| Number  | Country       | Date          |
|---------|---------------|---------------|
| 361,362 | Great Britain | Nov. 16, 1931 |

#### OTHER REFERENCES

70 Jour. of the Am. Pharm. Assoc. (Scientific edition), for February 1945, pages 56, 57, 58.

"Atlas Spans and Tweens," published by Atlas Powder Co., Wilmington, Del., November 1942, pages 5 and 8.

Rayon Textile Mo. for June, 1945, page 97.